

## UNITED STATES PATENT OFFICE

WILLOUGHBY STATHAM SMITH, OF BENCHAMS, NEWTON POPPLEFORD, HENRY JOSEPH GARNETT, OF LYME, SOLEFIELDS, SEVENOAKS, AND WALTER FREDERICK RANDALL, OF EWELL, ENGLAND, ASSIGNORS TO TELEGRAPH CONSTRUCTION AND MAINTENANCE COMPANY, LIMITED, OF LONDON, ENGLAND, AND DEUTSCH-ATLANTISCHE TELEGRAPHENGESELLSCHAFT, OF BERLIN, GERMANY

## MAGNETIC ALLOY

No Drawing. Application filed July 11, 1932, Serial No. 622,012, and in Great Britain July 22, 1931.

This invention relates to magnetic alloys of the nickel-iron class having a high permeability at low magnetizing forces, such as used for loading telephone and telegraph

5 conductors or the like in electrical circuits.

The invention is a development of the invention set forth in U. S. Patent 1,873,155, issued to Bernhard Scharnow, August 23, 1932, which concerns the incorporation of a 10 small percentage of a slightly-soluble element, i. e. one which does not readily form mixed crystals with the nickel-iron complex brought into solution at a high temperature, kept in supersaturated solution by rapid 15 cooling and separated in a very finely divided state by prolonged heating at a comparatively low temperature. The coercive force of the nickel-iron alloy is thereby increased and the permeability curve in the 20 range of small field strengths flattened.

For the continuous loading of signalling conductors, particularly in submarine telephone cables, it is desirable that the magnetic material should not only exhibit as constant 25 a permeability as possible under the conditions prevailing in the immediate neighbourhood of the conductor during signalling, as well as low hysteresis losses, but it should also have a high specific resistance in order 30 to diminish the eddy current losses occurring in the magnetic material during signalling. Further the mechanical properties of the metal must be such that it can be brought into the form of thin tape or fine wire.

35 The present invention aims to produce workable magnetic alloys having not only a high degree of constancy of permeability in weak magnetic fields, but also a high specific resistance.

40 According to the invention there is incorporated into the alloy a resistance-increasing element which passes into solid solution in the nickel-iron complex as well as the small percentage of the slightly-sol-

45 uble constituent which latter, or some of it, when the alloy is annealed at a high temperature, cooled rapidly from the annealing temperature or from an intermediate temperature, and then soaked at a comparatively low 50 temperature for a substantial period of time,

is precipitated out of solid solution in a finely divided state.

The term "a resistance-increasing element" used in this specification and the appended claims is intended to include one or more elements of the group, known to have the property of increasing the resistance of nickel-iron magnetic alloys, which comprises, chromium, molybdenum, tungsten, manganese, copper, aluminium, silicon, vanadium, cobalt.

It is not possible to state precise limits for the proportions of chromium, etc. to be incorporated because these would vary according to the extent of solid solubility in the particular nickel-iron complex employed. As a general guide the upper limits may be stated to be, for chromium (15%), molybdenum (12%), manganese (12%), tungsten (10%), copper (15%), aluminium (5%), silicon (5%), vanadium (5%), and cobalt (15%).

It must further be understood that the nature and amount of the above mentioned soluble constituents will govern the optimum 75 amount; and in some cases the choice, of the slightly soluble constituent to be added for producing the best working properties.

Examples of a suitable slightly soluble element are silver, beryllium, antimony, magnesium, calcium, phosphorous, sulphur, carbon. It is to be understood that an alloy produced according to the invention may incorporate one or more of these elements.

It is of advantage in some cases to anneal at a higher temperature than 900° C., for example at 1,000° C. or slightly above, since the absolute value of the permeability in its range of substantial constancy can thereby be raised. The rapid cooling may be immediately from the annealing temperature or from an intermediate temperature, e. g. 650° C., the previous cooling to the latter temperature being at a slower rate.

It will be understood in relation to the incorporation of the slightly-soluble constituent that, in determining the amount to add, due regard should be paid to what (e. g. sulphur or phosphorous) may already be present in the nature of accidental impuri-

55

65

70

75

80

85

90

95

100

ties. The proportion of certain elements, notably sulphur, phosphorus and zirconium, required to produce, after the heat-treatment, the desired flattening of the  $\mu$ /H curve 5 in the range of small field strengths is quite small; further the presence of certain elements, such as sulphur or phosphorus, in excess of a certain small proportion dependent upon the composition of the alloy, leads 10 to the production of brittle alloys. In exceptional cases it may happen that impurities of the desired kind are present in excess of the desired amount—or alternatively 15 the impurity may have a deleterious effect on the further constituents that it is desired to add—and there may then have to be applied a purifying treatment to bring about the necessary adjustment (including, it may be, the elimination or reduction of unwanted 20 constituents) before carrying out the annealing, quenching and soaking.

The invention is illustrated by the following table of examples (the rows 1(a), 25 2(a), etc. being inserted for comparison purposes) :—

| 30 | Composition (parts by weight)                                                                                       | Heat treatment                                                                             | Specific resistance (microhms per cm <sup>2</sup> ) | Initial permeability ( $\mu_0$ ) | Coefficient of permeability variation ( $(\mu_0.1 - \mu_0) / \mu_0$ ) |
|----|---------------------------------------------------------------------------------------------------------------------|--------------------------------------------------------------------------------------------|-----------------------------------------------------|----------------------------------|-----------------------------------------------------------------------|
|    | (1)                                                                                                                 | (a)                                                                                        |                                                     |                                  |                                                                       |
| 35 | Nickel..... 76.9<br>Iron..... 17.77<br>Manganese... 0.73<br>Molybdenum... 3.0<br>Silver..... 1.52                   | Annealed (1 hour) at 1000° C., slowly cooled (4 hours) to 600° C. and then rapidly cooled. | 46.0                                                | 4660                             | 0.0666                                                                |
| 40 |                                                                                                                     | (b)                                                                                        |                                                     |                                  |                                                                       |
|    |                                                                                                                     | Same as (a) followed by 36 hours' soaking at 375° C.                                       | 47.0                                                | 3160                             | 0.0150                                                                |
|    | (2)                                                                                                                 | (a)                                                                                        |                                                     |                                  |                                                                       |
| 45 | Nickel..... 77.2<br>Iron..... 17.77<br>Silver..... 0.94<br>Manganese... 0.8<br>Molybdenum... 3.0                    | Annealed (1 hour) at 1000° C., slowly cooled (4 hours) to 600° C. and then rapidly cooled. | 49.3                                                | 7370                             | 0.1600                                                                |
| 50 |                                                                                                                     | (b)                                                                                        |                                                     |                                  |                                                                       |
|    |                                                                                                                     | Same as (a) followed by 36 hours' soaking at 375° C.                                       | 50.5                                                | 4280                             | 0.0187                                                                |
|    | (3)                                                                                                                 | (a)                                                                                        |                                                     |                                  |                                                                       |
| 55 | Nickel..... 78.5<br>Iron..... 18.0<br>Molybdenum... 3.0<br>Manganese... 1.0<br>Silicon..... 2.0<br>Beryllium... 1.2 | Annealed (1 hour) at 1000° C., slowly cooled (4 hours) to 600° C. and then rapidly cooled. | 50.5                                                | 982                              | 0.0161                                                                |
| 60 |                                                                                                                     | (b)                                                                                        |                                                     |                                  |                                                                       |
|    |                                                                                                                     | Same as (a) followed by 5 hours' soaking at 375° C.                                        | 51.0                                                | 880                              | 0.0000                                                                |

What we claim is:—

1. The process of producing magnetic alloys of the nickel-iron class suitable for use in loading signalling conductors being workable to shape as desired and having high 70 specific resistance and low coefficient of permeability variation, which process comprises the incorporation into solid solution in the alloy of a resistance-increasing element and also the incorporation of a small percentage of a slightly soluble element, heating the alloy and quenching it from a high temperature so as to obtain a condition of supersaturation of the slightly soluble element in solid solution and thereafter soaking the 80 material at a lower temperature for a substantial period of time in order to precipitate some of that element out of solution in a finely divided state.

2. The process of producing magnetic alloys of the nickel-iron class suitable for use in loading signalling conductors being workable to shape as desired and having high specific resistance and low coefficient of permeability variation, which process comprises 90 the incorporation into solid solution in the alloy of a resistance-increasing element and also the incorporation of a small percentage of a slightly soluble element, heating the alloy to an annealing temperature, quenching so as to obtain a condition of supersaturation of the slightly soluble element in solid solution, and thereafter soaking the material between about 300° and 500° C. for a substantial period of time in order to precipitate some of that element out of solution in a finely divided state.

3. The process of producing magnetic alloys of the nickel-iron class suitable for use in loading signalling conductors being workable to shape as desired and having high specific resistance low coefficient of permeability variation, which process comprises the incorporation into solid solution in the alloy of a resistance-increasing element and 105 also the incorporation of a small percentage of a slightly soluble element, heating the alloy to an annealing temperature, cooling rather slowly to a lower temperature, such for example as 600° C. quenching so as to obtain a condition of supersaturation of the slightly soluble element in solid solution, and thereafter soaking the material between about 300° and 500° C. for a substantial 110 period of time in order to precipitate some of that element out of solution in a finely divided state.

4. A magnetic alloy of the nickel-iron class which is non-brittle and suitable for use in loading signalling conductors, having a high specific resistance and an adequately high initial permeability coupled with a low coefficient of permeability variation and which contains a resistance-increasing element in solid solution and a small 125

percentage of a slightly-soluble element out of solid solution and disseminated in a finely divided state throughout the mass of the alloy.

5. A magnetic alloy as claimed in claim 4, silver being specified as the slightly-soluble element.

6. A magnetic alloy as claimed in claim 4, beryllium being specified as the slightly-soluble element.

In testimony that we claim the foregoing as our invention we have signed our names this 30th day of June 1932.

15 WILLOUGHBY STATHAM SMITH.  
HENRY JOSEPH GARNETT.  
WALTER FREDERICK RANDALL.

20

25

30

35

40

45

50

55

60

65